

1,203,372.

F. J. LYSTER.  
SEPARATION OF METALLIC SULFID ORES,  
APPLICATION FILED MAY 8, 1913.

Patented Oct. 31, 1916.  
2 SHEETS—SHEET 1.



Fig. 1.

WITNESSES:

John C. Sanders  
Albert F. Neuman

INVENTOR

Henry James Lyster  
by  
John Mallaw White

ATTY

F. J. LYSTER.

## SEPARATION OF METALLIC SULFID ORES.

APPLICATION FILED MAY 8, 1913.

1,203,372.

Patented Oct. 31, 1916.

2 SHEETS—SHEET 2.



Witnesses:

W. M. Alcorn  
and Ashley Kelley

Inventor

Henry James Lyster  
By his Attorney  
Henry K. Williams

# UNITED STATES PATENT OFFICE.

FLEURY JAMES LYSTER, OF BROKEN HILL, NEW SOUTH WALES, AUSTRALIA, ASSIGNOR,  
BY MESNE ASSIGNMENTS, TO MINERALS SEPARATION AMERICAN SYNDICATE (1913)  
LIMITED, OF LONDON, ENGLAND.

## SEPARATION OF METALLIC SULFID ORES.

1,203,372.

Specification of Letters Patent.

Patented Oct. 31, 1916.

Application filed May 8, 1913. Serial No. 766,346.

*To all whom it may concern:*

Be it known that I, FLEURY, JAMES LYSTER, subject of the King of Great Britain and Ireland, residing at Broken Hill, in the State of New South Wales, Commonwealth of Australia, mill foreman, have invented certain new and useful Improvements in or Relating to the Separation of Metallic Sulfid Ores, of which the following is a specification.

This invention relates to certain improvements in the separation of minerals and particularly of mixed zinc and lead sulfid ores.

The object of this invention is to separate metalliferous portions of an ore, such for example, as the sulfid of lead (galena) from other portions of the ore, as by a method of differential or selective flotation—separation of lead sulfid (galena) and zinc sulfid (blende) obtaining products relatively rich in lead on the one hand, and a zinc product relatively low in lead on the other hand.

The flotation separation process employed is preferably the agitation-froth process of the general type described in United States Patents No. 835,120 to Sulman, Picard and Ballot, of November 6, 1906, No. 955,012 to H. L. Sulman, of April 12, 1910, No. 962,678 to Sulman, Greenway and Higgins, of June 28, 1910, No. 1,064,723 to Greenway and Lavers, of June 17, 1913, and British Patent No. 18,943 of 1910 to Minerals Separation, Limited, as a communication from H. H. Greenway.

Further this invention is a development of that described in the previous United States Patent No. 1,067,485 to Nutter and Lavers, of July 15, 1913, that is to say, a separation is effected between the different metallic sulfids in the agitation-froth process by varying the controlling conditions and particularly the chemical constitution of the solution employed.

I have discovered that sulfid of lead (galena) may be separated from sulfid of zinc (blende) without any preliminary treatment by subjecting the ore or metalliferous materials to a flotation separation treatment at a low temperature with eucalyptus oil or other frothing agent and with agitation or aeration in a neutral or alkaline, but not an acid, solution of the sulfates, chlorides or nitrates of calcium, magnesium, sodium, potassium or mixtures of

these substances. I have also discovered that neutral or alkaline, but not acid, solutions of other suitable substances can be employed such as sulfate of manganese, zinc, or iron, chlorid of barium, carbonate and bicarbonate of sodium or potassium or mixtures of these substances.

The suitability of any given substance in a neutral or alkaline solution can be easily determined by a laboratory test as herein-after described.

I have found that mineralized water such as is obtained from the underground working at Broken Hill, Australia is a suitable solution for carrying out my process. Such water gives approximately the following analysis:—

|                             | Gr. per gall. |
|-----------------------------|---------------|
| Total soluble solids        | 666           |
| Volatile and organic matter | 57.2          |
| Silica                      | 2.2           |
| Calcium oxid                | 78.2          |
| Magnesium oxid              | 53.           |
| Sulfur trioxid              | 205.          |
| Chlorin                     | 178.          |
| Manganese                   | 30.3          |
| Zinc                        | 5.            |
| Alumina                     | 4.            |
| Carbon dioxide              | 9.3           |
|                             | 622.2         |
|                             | 80            |

and is alkaline in reaction when submitted to the usual test with methyl orange.

In carrying this process into effect a plant similar to that employed in and common to flotation "frothing" processes is employed, but the plant I recommend is illustrated in the accompanying drawings in which—

Figure 1 is a longitudinal elevation and Fig. 2 a cross section of a unit with the supply devices in elevation. Fig. 3 is a sectional elevation of an apparatus suitable for testing.

I will now describe my process as carried out in the apparatus shown in Figs. 1 and 2.

The ore is first ground to a suitable degree of fineness (preferably to slimes so that the different metallic sulfid particles are disassociated from each other). This finely ground ore with its accompanying circuit water (which is a solution such as herein-before described) is led into a settler or thickener A to remove excess water. The thickened pulp is then led into a vessel B from which it passes to the first centrifugal pump C<sup>1</sup> of series C<sup>1</sup>, C<sup>2</sup>, C<sup>3</sup>, C<sup>4</sup>, C<sup>5</sup>, C<sup>6</sup>. These centrifugal pumps are each connected to the individual members of a corresponding series of separating boxes D', D<sup>2</sup>, D<sup>3</sup>, D<sup>4</sup>,

- D<sup>5</sup>, D<sup>6</sup>. These centrifugal pumps act as agitators or mixers and means are provided (such as an inlet pipe E) for feeding in the requisite amount of eucalyptus oil or other frothing agent, about 2 lbs. per ton of material treated, as well as the requisite amount of air (such as by a tap F) into the suction pipe G' thereof which is connected to the feed vessel B. The centrifugal pump 16 C<sup>1</sup> draws in pulp, air, and frothing agent and produces an intimate mixture which is discharged through the outlet pipe H to the separator box D', the delivery of the pump being controlled by the admission of 15 air by the tap F. The particles of lead sulfid (galena) are found to rise to the top of the separator box D' where an inverted pyramid J' diverts the froth toward the discharge lip or launder K' from which it 20 flows to the receptacle for settling and collecting the lead concentrate. The particles which do not rise or float, together with the balance of the water, sink to the bottom of the box D' and are there withdrawn by the 25 outlet pipe L' which is connected to the suction pipe G<sup>2</sup> of the next pump C<sup>2</sup> of the series and the operation is repeated, the residues of one separator box D' passing to the centrifugal pump C of the next in series. 30 In the plant illustrated in the accompanying drawings there are six separator boxes and their attendant pumps which comprise one series or unit, but it will be understood that this number is dependent upon the proportion of mineral contained in the ore and the degree of agitation and aeration required, the repetition of the operations being carried on until the grade of the concentrates becomes too low in lead and the zinc 35 begins to appear therein. The temperature I prefer is below 100° F. that is to say the operation is conducted at the ordinary temperature and no extraneous heat is utilized. 40 I have observed in working the process that an excessive alkalinity tends to retard the selective flotation of the lead sulfid particles. Therefore if the solution be alkaline the same should be only slightly alkaline but sufficient to respond to the well known 45 methyl orange test when the process is employed for the selective separation of lead sulfid.
- The suitability of the substances hereinbefore indicated and the proportion thereof 50 to the solution and the degree and duration of agitation or aeration of the material treated can be determined in a laboratory test which may be conducted as follows in an apparatus as illustrated in Fig. 3 of the 55 accompanying drawings which shows a side sectional elevation. This apparatus comprises an agitating or mixing vessel N having a rotating impeller O, a separating box P on the side thereof connected to the 60 mixer by a passage R, and by a flexible hose 65 or pipe S at the bottom. In carrying out a test the mixing vessel N contains the solution which corresponds with the circuit water of the working plant, and eucalyptus oil or other frothing agent is then added in measured quantities. The impeller O is then 70 rotated at about 1700 revolutions per minute and a charge of about 448 grams of ore is fed in. Sufficient solution is added to fill the separating box P to the level of its discharge lip. The agitated pulp is forced through the passage R into the separating box P and the "float" or "froth" rising to the surface is skimmed off over the lip. The pulp is continuously circulated by being drawn from the bottom of the box P by the pipe S back into the mixer N by the action of the impeller O. The flotation is continued until the "float" or "froth" is noticed by observation to become lower in lead and the zinc begins to appear therein. The appearance of the concentrate being skimmed off over to the lip of the separating box will indicate the duration of agitation necessary to obtain a good concentrate combined with a good recovery while experience will indicate the amount of frothing agent necessary and further quantities may be added at intervals as found necessary. The residue is run off from the bottom of the machine by disconnecting the flexible hose or pipe S. Repeated trials with different solutions and with different strengths will indicate what is best suited to the particular ore under treatment. The ascertained duration of agitation and aeration will govern the number of separator boxes which will be necessary in the working plant when that hereinbefore described is used. 95
- The following examples are given of solutions which have been used by me in obtaining a selective separation of the lead sulfids from the zinc sulfids in what are known as calcitic slimes at Broken Hill to which my process is peculiarly well suited averaging about eleven (11) per cent. of zinc and about thirteen (13) per cent. of lead using about from 2 to 5 lbs. of eucalyptus oil per ton. 105
- |                   |     |                    |     |
|-------------------|-----|--------------------|-----|
| Calcium sulfate   | 160 | grains per gallon. | 115 |
| { Calcium sulfate | 160 | "                  |     |
| with              |     |                    |     |
| { Calcium hydrate | 1.8 | "                  | "   |
| { Calcium sulfate | 160 | "                  | "   |
| with              |     |                    |     |
| { Calcium hydrate | 3.6 | "                  | "   |
| Calcium chlorid   | 300 | "                  | "   |
| { Calcium chlorid | 300 | "                  | "   |
| with              |     |                    | 120 |
| { Calcium hydrate | 1.8 | "                  | "   |
| { Calcium chlorid | 300 | "                  | "   |
| with              |     |                    |     |
| { Calcium hydrate | 3.6 | "                  | "   |
| Calcium nitrate   | 300 | "                  | "   |
| { Calcium nitrate | 300 | "                  | "   |
| with              |     |                    | 125 |
| { Calcium hydrate | 1.8 | "                  | "   |
| { Calcium nitrate | 300 | "                  | "   |
| with              |     |                    |     |
| { Calcium hydrate | 3.6 | "                  | "   |
| { Calcium nitrate | 300 | "                  | "   |
| with              |     |                    |     |
| { Calcium hydrate | 18  | "                  | "   |

|    |                          |     |                    |
|----|--------------------------|-----|--------------------|
|    | Magnesium sulfate        | 400 | grains per gallon. |
|    | { Magnesium sulfate with | 400 | " "                |
|    | Calcium hydrate          | 1.8 | " "                |
|    | { Magnesium sulfate with | 400 | " "                |
|    | Calcium hydrate          | 3.6 | " "                |
| 5  | { Magnesium sulfate with | 400 | " "                |
|    | Calcium hydrate          | 18  | " "                |
|    | Magnesium chlorid        | 300 | " "                |
|    | { Magnesium chlorid with | 300 | " "                |
|    | Calcium hydrate          | 1.8 | " "                |
| 10 | { Magnesium chlorid with | 300 | " "                |
|    | Calcium hydrate          | 3.6 | " "                |
|    | Magnesium nitrate        | 300 | " "                |
|    | { Magnesium nitrate with | 300 | " "                |
|    | Calcium hydrate          | 1.8 | " "                |
| 15 | { Magnesium nitrate with | 300 | " "                |
|    | Calcium hydrate          | 3.6 | " "                |
|    | Magnesium nitrate        | 300 | " "                |
|    | { Magnesium nitrate with | 300 | " "                |
|    | Calcium hydrate          | 18  | " "                |
| 20 | Sodium chlorid           | 800 | " "                |
|    | { Sodium chlorid with    | 800 | " "                |
|    | Calcium hydrate          | 1.8 | " "                |
|    | { Sodium chlorid with    | 800 | " "                |
|    | Calcium hydrate          | 3.6 | " "                |
| 25 | { Sodium chlorid with    | 800 | " "                |
|    | Calcium hydrate          | 18  | " "                |
|    | Potassium sulfate        | 300 | " "                |
|    | { Potassium sulfate with | 300 | " "                |
|    | Calcium hydrate          | 1.8 | " "                |
|    | Potassium chlorid        | 800 | " "                |
| 30 | { Potassium chlorid with | 800 | " "                |
|    | Calcium hydrate          | 1.8 | " "                |
|    | { Potassium chlorid with | 800 | " "                |
|    | Calcium hydrate          | 3.6 | " "                |
| 35 | { Potassium chlorid with | 800 | " "                |
|    | Calcium hydrate          | 18  | " "                |
|    | Potassium nitrate        | 400 | " "                |
|    | { Potassium nitrate with | 400 | " "                |
|    | Calcium hydrate          | 1.8 | " "                |
| 40 | { Potassium nitrate with | 400 | " "                |
|    | Calcium hydrate          | 18  | " "                |
|    | Barium chlorid           | 300 | " "                |
|    | { Barium chlorid with    | 300 | " "                |
|    | Calcium hydrate          | 1.8 | " "                |
| 45 | { Barium chlorid with    | 300 | " "                |
|    | Calcium hydrate          | 3.6 | " "                |
|    | Sodium sulfate           | 800 | " "                |
|    | { Sodium sulfate with    | 800 | " "                |
|    | Calcium hydrate          | 1.8 | " "                |
| 50 | { Sodium sulfate with    | 800 | " "                |
|    | Calcium hydrate          | 3.6 | " "                |
|    | { Sodium sulfate with    | 800 | " "                |
| 55 | Calcium hydrate          | 18  | " "                |
|    | Sodium bicarbonate       | 600 | " "                |
|    | Sodium carbonate         | 500 | " "                |
|    | Manganese sulfate        | 300 | " "                |
|    | Zinc sulfate             | 500 | " "                |
|    | Ferrous sulfate          | 300 | " "                |
|    | Alum                     | 300 | " "                |

I have further discovered that the residues obtained as before described containing the bulk of the zinc sulfids may be further treated by flotation separation to produce a concentrate rich in zinc by first dewatering and thickening the pulp and then submitting it to a repetition of the flotation separation, using however fresh water in lieu of the solution previously employed, or by further

continuing the process hereinbefore described, after the recovery of the lead sulfids (galena) in a separate de-zincing unit until the zinc sulfids (blende) appear upon the surface of the solution and are carried over into the launders hereinbefore mentioned. In operation I prefer the former to the latter method for the recovery of the zinc sulfids (blende). In this way a zinc concentrate may be obtained and thereby both the lead sulfids and zinc sulfids recovered in separate products by flotation separation without recourse to separation by gravitation, tables or vanners as heretofore.

Where the term "abnormal amount" is employed in the following claims with reference to the salts in solution it is intended to mean that the amount of salts present is in excess of that ordinarily found in natural fresh water.

I claim:

1. A process for the separation of lead sulfid from zinc sulfid in ores containing mixed lead and zinc sulfids, which consists in subjecting the said ores to a flotation separation treatment by agitating them with a frothing agent in a non-acid solution of the mineral acid salts of metals which form basic hydroxids, and thereby separating the lead sulfid from the zinc sulfid.

2. A process for the separation of lead sulfid from zinc sulfid in ores containing mixed lead and zinc sulfids, which consists in subjecting the said ores to a flotation separation treatment by agitating them with a frothing agent in a slightly alkaline solution of the mineral acid salts of metals which form basic hydroxids, and thereby separating the lead sulfid from the zinc sulfid.

3. A process for the separation of minerals which consists in subjecting a pulp of an ore containing mixed minerals to agitation and aeration with a small proportion of a frothing agent in a non-acid solution containing in abnormal amount a plurality of the mineral acid salts of metals which form basic hydroxids so as, by such agitation and aeration, to produce a froth of concentrates, said solution being non-acid during separation of the minerals, and separating the froth.

4. A process for the separation of minerals which consists in subjecting a pulp of an ore containing mixed minerals to agitation and aeration with a small proportion of a frothing agent in a slightly alkaline solution containing in abnormal amount a plurality of the mineral acid salts of metals which form basic hydroxids so as, by such agitation and aeration, to produce a froth of concentrates, said solution being alkaline during separation of the minerals, and separating the froth.

5. A process for the separation of lead

- sulfid from zinc sulfid in ores containing mixed lead and zinc sulfids, which consists in subjecting the said ores to a flotation separation treatment by agitating them with 5 eucalyptus oil in a non-acid solution of the mineral acid salts of metals which form basic hydroxids, and thereby separating the lead sulfid from the zinc sulfid.
6. A process for the separation of lead sulfid from zinc sulfid in ores containing mixed lead and zinc sulfids, which consists in subjecting the said ores to a flotation separation treatment by agitating them with eucalyptus oil in a slightly alkaline solution 10 of the mineral acid salts of metals which form basic hydroxids, and thereby separating the lead sulfid from the zinc sulfid.
7. A process for the separation of minerals which consists in subjecting a pulp of an ore containing mixed minerals to agitation and aeration with a small proportion of a frothing agent in a non-acid solution containing in abnormal amount the sulfates and chlorids of calcium, magnesium and manganese, so as, by such agitation and aeration, to produce a froth of concentrates, and separating the froth. 15
8. A process for the separation of minerals which consists in subjecting the pulp of an ore containing mixed minerals to agitation and aeration with a small proportion of a frothing agent in a slightly alkaline solution containing in abnormal amount the sulfates and chlorids of calcium, magnesium and manganese, so as, by such agitation and aeration, to produce a froth of concentrates, and separating the froth. 20
9. A process for the separation of lead sulfid from zinc sulfid in ores containing mixed lead and zinc sulfids, which consists in subjecting the said ores to a flotation separation treatment at about atmospheric temperature by agitating them with a frothing agent in a non-acid solution of the mineral acid salts of metals which form basic hydroxids, thereby separating the lead sulfid 25
- from the zinc sulfid and obtaining a concentrate relatively rich in lead.
10. A process for the separation of lead sulfid from zinc sulfid in ores containing mixed lead and zinc sulfids, which consists in subjecting the said ores to a flotation separation treatment by agitating them with a frothing agent in a non-acid solution containing the sulfates and chlorids of calcium, magnesium and manganese, thereby separating the lead sulfid from the zinc sulfid. 30
11. A process for the separation of lead sulfid from zinc sulfid in ores containing mixed lead and zinc sulfids, which consists in subjecting the said ores to a flotation separation treatment by agitating them with a frothing agent in a slightly alkaline solution containing the sulfates and chlorids of calcium, magnesium and manganese, thereby separating the lead sulfid from the zinc sulfid. 35
12. A process for the separation of lead sulfid from zinc sulfid in ores containing mixed lead and zinc sulfids, which consists in subjecting the said ores to a flotation separation treatment by agitating them with eucalyptus oil in a non-acid solution containing the sulfates and chlorids of calcium, magnesium and manganese, thereby separating the lead sulfid from the zinc sulfid. 40
13. A process for the separation of lead sulfid from zinc sulfid in ores containing mixed lead and zinc sulfids, which consists in subjecting the said ores to a flotation separation treatment by agitating them with eucalyptus oil in a slightly alkaline solution containing the sulfates and chlorids of calcium, magnesium and manganese, thereby separating the lead sulfid from the zinc sulfid. 45
- In testimony whereof I have affixed my signature in presence of two witnesses.
- FLEURY JAMES LYSTER.
- Witnesses:
- EDWARD JOHN TURNER,  
CHARLES STANLEY BURGESS.